

July 9, 1968

P. S. McDERMOTT ETAL

3,392,066

METHOD OF VAPOR GROWING A HOMOGENEOUS MONOCRYSTAL

Filed Dec. 23, 1963

2 Sheets-Sheet 1

FIG. 2



FIG. 1



INVENTORS  
PHILIP S. McDERMOTT  
GERALD W. MANLEY  
RALPH J. RILEY  
LAWRENCE R. YETTER

BY

*John S. Smith*  
ATTORNEY

July 9, 1968

P. S. McDERMOTT ET AL

3,392,066

METHOD OF VAPOR GROWING A HOMOGENEOUS MONOCRYSTAL

Filed Dec. 23, 1963

2 Sheets-Sheet 2



FIG. 4



FIG. 5



FIG. 3

1

3,392,066

**METHOD OF VAPOR GROWING A HOMOGENEOUS MONOCRYSTAL**

Philip S. McDermott, Athens, Pa., and Gerald W. Manley, Oneonta, and Ralph J. Riley and Lawrence R. Yetter, Apalachin, N.Y., assignors to International Business Machines Corporation, New York, N.Y., a corporation of New York

Filed Dec. 23, 1963, Ser. No. 332,563  
7 Claims. (Cl. 148—175)

**ABSTRACT OF THE DISCLOSURE**

A halogen transport process carried on in an evacuated chamber containing a growth receiving substrate and ingots of source materials together with iodine vapor. Two independently coolable heat sinks permit separate control of the temperature of the substrate and source regions of the chamber. The process involves first causing vapor transport from the substrate to the source (by controlling the temperature differential between source and substrate areas) to cleanse the growth receiving surface of the substrate. Thereafter, the process is reversed and growth is deposited on the substrate. High quality growth is achieved by maintaining substrate temperature just above the temperature at which a condensate is produced on the substrate. The vapor growth process produces high quality monocrystals of III and V valence group elements. Semiconductor devices fabricated from such crystals exhibit spontaneous and stimulated emission of radiation in the 0.9 to 3.2 micron range of wavelengths.

The process provides monocrystals of controllable composition within the system  $\text{In}(\text{As}_x\text{P}_{1-x})$ .

In recent years, considerable effort has been directed toward the investigation of radiation emission characteristics of various devices, and particularly to the phenomenon of stimulated emission of radiation. Devices which exhibit the capability of stimulated emission of radiation in the infrared, visible or ultraviolet regions of the radiation spectrum are known as "lasers" (an acronym derived from "light amplification by stimulated emission of radiation"). Devices of this type are capable of producing radiation which is highly directional, coherent, and monochromatic. They have received wide publicity in the past several years. Utility for lasers has been found in various areas, for example, in the fields of communication, object detection and ranging, and data handling. In addition, these devices appear to have considerable utility as sources of destructive force.

Of lesser prominence, but also important, are devices which exhibit the characteristic of spontaneous emission of radiation. The radiation provided by spontaneous emission is not as highly coherent as stimulated emission, nor is it as monochromatic. Spontaneously emitted radiation or "fluorescence" is, however, of generally narrow bandwidth and it is highly useful, for example, for short range communication, etc.

The establishment of spontaneous and stimulated emission of radiation involves the creation of an artificial distribution of electrons at energy levels other than the natural distribution in a host environment through the application of energy, known as pumping energy, to the host environment. This artificial distribution of electrons at higher than normal energy levels results in a greater fraction of filled energy states at the higher levels than at the lower levels. The electrons present in the artificial distribution at higher than normal levels eventually give up their energy and undergo a transition to their normal levels. The energy released by this action takes the form of photons emitted from the device.

2

In the case of spontaneous emission, the photons are emitted in a plurality of modes and the fluorescence emitted from the device covers a range of wavelengths which, while narrow, is considerably wider than that observed in the case of stimulated emission. A plot of wavelengths vs. light intensity shows a generally Gaussian or "bell shaped" distribution covering a range of, perhaps, 0.01 micron. The band of emitted wavelengths is commonly referred to as the emitted "line." The line is said to have a width which is essentially the difference in wavelength between the half power points of the distribution curve. The line has a central wavelength at which maximum output radiation intensity is observed and this is known as the "line maximum" wavelength.

Spontaneous emission is a radiative process in which the energy transitions that result in photon emission are not necessarily influenced by the presence of other similar photons. As the pumping energy is increased, emission of photons in one mode begins to occur at the expense of other modes. It appears that emitted photons strike excited atoms and influence the emission of additional photons in fixed phase relation so that mode selectivity is achieved. This phenomenon, which is evidenced by a substantial narrowing of the emission line as well as an increase in coherency and directionality of the output radiation, is known as stimulated emission.

The host environment in which the radiation is produced may take any of several forms. In laser devices currently available in the art the host environment may be either a gas, such as helium-neon mixture or it may be a crystal of one of several different compositions. The emission has been produced by pumping energy in the form of light or, in the case of crystals of semiconductor material, the pumping energy may be supplied by injecting electrons into the semiconductor. It is toward the devices of the semiconductor type that the present invention is directed.

Spontaneous and stimulated emission of radiation from semiconductive materials is achieved by providing in the material a p-n junction and injecting minority carriers across the junction in a forward bias direction in appropriate density. The emission is produced by the mechanism previously described in response to carrier recombination via the junction. No attempt will be made here to describe in detail the precise occurrences which result in production of radiation by carrier injection in semiconductor diode devices. A detailed explanation of the phenomena may be found in several recent articles, for example "Semiconductor Lasers," by B. Lax in *Science*, vol. 141, No. 3587, Sept. 27, 1963, pp. 1247-1255. Other references are cited in the copending application, Ser. No. 230,607, by Burns et al., filed Oct. 15, 1962 and assigned to the assignee hereof.

Spontaneous and stimulated emission of radiation has been observed in semiconductor diodes of several compounds of elements in the III and V valence groups, such as gallium arsenide, indium arsenide, indium phosphide, and more recently gallium arsenide phosphide and indium gallium arsenide. The wavelength of the emission from diode devices is a function of the composition and in the case of most of those compounds mentioned above, is observed to be in the sub-micron range.

It is desirable to have the capability of producing spontaneous and stimulated emission at controlled wavelengths over a broad range. Moreover, it is desirable to provide devices capable of producing emission at wavelengths which correspond to favorable transmission regions of the spectrum in the atmosphere. These favorable regions are commonly known as "atmospheric windows" and they exist at various points in the radiation spectrum. Three such "windows" of interest to the present invention are found in the infrared region of the spectrum at

wavelengths of about 1.25 microns, 1.6 microns, and 2.25 microns.

According to this invention there are provided means and methods for providing homogeneous single crystals structures of controlled composition within predetermined limits of a quality and perfection adequate for realization of spontaneous and stimulated emission over a generally broad range of wavelengths in the infrared portion of the spectrum including the portion containing the windows mentioned above.

It has been found that by means of a novel vapor growth process, compounds embodying III-V elements may be provided in the form of homogeneous single crystals of high quality and perfection. Moreover, it has been found that by means of this process, the composition of the final compound can be controlled within relatively close tolerances so that devices capable of producing emission at predetermined wavelengths can be fabricated.

This novel process has been employed to provide homogeneous single crystal compounds of controlled composition in the system of  $In(As_xP_{1-x})$ , hitherto unknown in this form. Devices fabricated from crystals of compositions in this system display emission wavelengths which vary from 0.9 micron (the emission wavelength of InP) to 3.2 microns (the emission wavelength of InAs).

Accordingly, it is a primary object of this invention to provide homogeneous single crystals of controlled composition and of quality and perfection adequate for use as spontaneous and stimulated emission sources.

Another object of the invention is to provide improved means and methods of growing homogeneous single crystals of controlled composition.

A further object of the invention is to provide an improved method for producing compounds of controlled composition within the system  $In(As_xP_{1-x})$  in the form of homogeneous single crystals of desired size.

Still another object of the invention is to provide means for growing homogeneous single crystals of controlled composition and for simultaneously doping said crystals with selected impurities.

Another primary object of the invention is to provide novel solid state devices for producing spontaneous and stimulated radiation in the infrared portion of the radiation spectrum.

It is also an object of this invention to provide novel solid state light sources of controlled frequency in the 0.9 to 3.2 micron range.

It is also an object of this invention to provide improved injection diodes for emitting radiation.

A further object of the invention is to provide injection diodes having output radiation wavelengths which correspond to favorable transmission regions or "atmospheric windows" in the infrared portion of the radiation spectrum.

The foregoing and other objects, features, and advantages of the invention will be apparent from the following more particular description of preferred embodiments of the invention, as illustrated in the accompanying drawings.

In the drawings:

FIG. 1 is a perspective view illustrating the crystal growing apparatus provided in accordance with this invention;

FIG. 2 is a longitudinal vertical sectional view taken through the reaction chamber which forms part of the apparatus of FIG. 1;

FIG. 3 is a diagrammatic illustration of an injection diode provided in accordance with this invention;

FIG. 4 is a graph showing the bandwidth of radiation produced in the cases of spontaneous and stimulated emission from a typical diode provided in accordance with this invention; and

FIG. 5 is a graph showing the correlation between radiation wavelength and composition for diodes provided in accordance with this invention.

The phenomena of spontaneous and stimulated emission of radiation have been observed in several semiconductive materials, as described hereinbefore. One of the characteristics of a semiconductive material necessary for the establishment of these phenomena is a homogeneous single crystal structure of high quality and perfection. According to this invention means and methods have been developed by which semiconductive compounds of elements in the III and V valence groups of the Mendeleeff periodic chart can be grown in the form of single crystals of desired size and of a quality and perfection suitable for establishment of spontaneous and stimulated emission. The means and methods of this invention have been employed to produce novel high quality homogeneous single crystals of controlled composition in the system  $In(As_xP_{1-x})$ .

The process by which crystals are grown in accordance with this invention is a vapor transport process by which elements are caused to be deposited by disproportionation reaction on a substrate from source materials at temperatures lower than the melting points of the elements involved. The principles of vapor growth and disproportionation reactions are known in the art and will not be discussed in detail herein. Detailed information on this subject is available in a group of five articles in the IBM Journal of Research and Development, vol. 4, No. 3, July 1960, at pages 248 through 279, and in the references listed in these articles. It is sufficient for an understanding of this invention to say simply that the disproportionation reaction involves the transport of materials in the form of vapor phase iodides (iodine being the transport agent) from source materials at one temperature to a receiving substrate at a lower temperature.

The improved vapor growing process of this invention is carried out with the apparatus shown in FIGS. 1 and 2 of the drawing. The apparatus includes a quartz chamber 10 having a generally semicylindrical outline with a flattened floor section 12. At one end of the chamber 10 a flat transparent quartz end wall 14 is fused to form a viewing window and to seal that end of the chamber. The opposite end is initially open to permit the various materials to be used in the growing process to be loaded. The chamber is evacuated and this end of the chamber is eventually sealed by fusing a quartz plug 16 in place, as shown in FIG. 2.

The reaction chamber 10 is arranged to have two temperature regions, as will be explained more fully later herein, and these are provided by attaching beneath the floor 12 of the chamber at spaced points a pair of metallic blocks 18 and 20 to act as heat sinks. The heat sinks 18 and 20 are held in place by bands 19 and 21 as shown. These heat sinks are preferably fabricated of a substance such as silver which has high conductivity and will withstand the temperature involved.

The heat sinks 18 and 20 have fluid conducting apertures 22 formed therein and fluid lines 24 and 26 are connected thereto to permit circulation of coolant, such as air, through the sinks. The fluid lines 24 and 26 are coupled to suitable circulating means (not shown) for pumping coolant through the heat sinks 18 and 20. The circulating means for the line 24 is independent of the means for the line 26 so that different temperatures can be maintained at the heat sinks 18 and 20. Temperature sensing means 28 and 30 are provided for accurately detecting the temperature of the heat sinks 18 and 20. In the embodiment shown in FIGS. 1 and 2 these sensing means are in the form of thermocouples contacting the metallic heat sinks. The thermocouples are connected to suitable temperature registering means (not shown).

The heat sinks 18 and 20 and their associated temperature control and indicating means provide two regions of variable temperature in the chamber 10. The region adjacent the sink 18 is a deposition region and that adjacent the sink 20 is a source region. Into the chamber immediately above the heat sink 18 is placed a substrate 32

upon which the crystal is to be grown, and above the heat sink 20 are placed pieces 34 and 36 of the materials which are to be used as sources.

To insure growth of a monocrystal of high quality and perfection the substrate 32 must be carefully prepared. It is essential that the substrate 32 be itself a monocrystal and that it be cut along crystallographic planes to provide a growth receiving surface 33 aligned along a desired plane. The substrate need not be of the same composition as the crystal to be grown thereon. The substrate should be of a material having a lattice spacing similar to that of the crystal to be grown.

In the growing processes performed in accordance with this invention substrates of monocrystal indium arsenide were used. These substrates were cut from monocrystal ingots previously aligned by X-ray techniques, to provide growth receiving surfaces along the (100) crystallographic plane. The receiving surface 33 of each substrate 32 is polished using a glass plate and an abrasive of 600 mesh SiC, and then buffed with an alcohol and bromide mixture on 0.1 micron grit polishing paper.

The donor or source pieces 34 and 36 are obtained as ingots including all of the elements to be combined in the deposited crystal. In growing crystals of the system  $In(As_xP_{1-x})$  ingots of InAs and InP are employed. The ingots may be polycrystalline and need not be cut along crystallographic planes. It has been found that the composition of the grown crystal is proportional to the respective areas of the ingot surfaces which face the substrate in the reaction chamber.

It appears that the etching of the source materials occurs primarily at these faces, although some etching of the top and side surfaces is also observed. The relation of face area to final composition is sufficient, however, to permit composition control to within tolerances in the order of a few percent. Accordingly, the source ingots 34 and 36 are cut so that the areas of faces 35 and 37 are in proportion to the desired composition of the final product. For example, if a crystal of  $In(As_{0.5}P_{0.5})$  is desired, the areas of the faces 35 and 37 of the ingots are made equal. If a crystal of  $In(As_{0.2}P_{0.8})$ , then the ingots 34 and 36 are cut so that the areas of faces 35 and 37 provide the ratio 2:8.

The source ingots 34 and 36 are polished with glass plates and 600 mesh SiC abrasive and cleaned with an alcohol bromide solution to insure that all surfaces thereof are regular and free of foreign material. They are then placed in the chamber 10 directly over the heat sink 20 with the surfaces 35 and 37 facing the substrate.

The crystal grown in the reaction chamber is simultaneously doped as it is grown, so it is necessary to provide in the chamber an amount of doping material. The doping material is chosen in accordance with the type of impurity desired in the crystal. For growing an n-type crystal a small piece of tellurium or other n-type dopant such as selenium, silicon, etc. is placed in the chamber. This substance will vaporize at the temperatures employed and a piece weighing between about 0.5 to 5 mg. in a 5 to 6 cubic centimeter chamber will provide a suitable impurity concentration of about  $4 \times 10^{19}$  carriers per cubic centimeter in the crystal.

The transport agent used is semiconductor grade iodine. Because of the low melting point of this substance, care must be exercised to avoid its being evaporated away during evacuation of the chamber 10. To prevent this, the chamber 10 is evacuated, by connection to the manifold of a vacuum pump (not shown), before the iodine is introduced. The iodine is placed in a separate vessel which is also connected to the manifold through a valve which is initially closed. After the chamber 10 has been evacuated to about  $10^{-7}$  torr., the manifold is valved off from the pump and the valve giving access to the iodine vessel is opened. The iodine vessel is small enough so that the air contained therein does not reduce the vacuum to less than about  $10^{-4}$  torr.

Once the iodine vessel is evacuated, it is immersed in liquid nitrogen to prevent sublimation of the iodine, and pumping is resumed to return the chamber to  $10^{-7}$  torr. Then the chamber is immersed in liquid nitrogen and the iodine vessel is gently heated to cause the iodine to be transferred to the chamber 10 by distillation. Following this, the plug 16 is fused in place to seal the chamber and the connection to the vacuum system is broken.

The iodine loading process just described is but one of several processes which may be employed for the purpose. Those familiar with the vapor growing art will recognize that other processes are also available.

After the reaction chamber has been loaded, evacuated, and sealed the heat sinks 18 and 20 are secured in place and the apparatus is placed in a furnace, for example, a clam shell furnace 38 is shown in FIG. 1. The furnace is closed and sealed to prevent undesirable air currents around the chamber 10. In sealing the furnace it is necessary to provide a viewing port to permit visual access to the chamber interior through the window 14. The viewing port may take the form of a quartz plate at the left end of the clam shell furnace 38.

The growth process is initiated by heating the furnace to a temperature of about  $830^{\circ}$  C. The furnace is held at this temperature for the duration of the process. During the heating process, the interior of the chamber 10 will be observed to take on first an iodine violet color and then the yellowish color characteristic of indium iodides.

As the temperature within the reaction chamber builds up the coolant controls for the heat sink 20 are operated to reduce the temperature of the source area. Sufficient coolant is circulated to maintain the source area about  $100^{\circ}$  C. below the ambient furnace temperature. The deposition region is not cooled appreciably. It may be maintained a few degrees below the ambient furnace temperature to provide for positive control in either direction. The purpose of cooling the source region is to produce some vapor transport from the substrate to the source to clean the surface 33, and to insure that any undesirable low temperature reaction products are condensed in the source region and do not contaminate the substrate. As the temperature increases above about  $500^{\circ}$  C. the upper surface of the substrate is observed to change texture and become substantially glossy. This change in appearance occurs in response to etching of the surface by the iodine vapor. This etching of the substrate surface cleans it in preparation for the subsequent deposition and is found to be necessary to insure growth of a high quality crystal. While etching commences with the surface of the substrate facing the source region, sufficient etching occurs at the surface 33 to clean it before the front is appreciably eaten away.

The pre-etching process does not require a substantial time and may be considered complete after about 10 minutes or when the substrate surface has taken on a uniform glossy appearance. The process will usually be complete by the time the furnace has reached  $800^{\circ}$  C. At this time, the supply of coolant to the source area heat sink 20 is diminished and it is allowed to approach the furnace temperature within a few degrees. At this time coolant is circulated through the heat sink 18 at the deposition region of chamber 10 to cool that area. As the temperature at the source region builds, substantial etching of the source ingots 34 and 36 is observed.

Coolant is supplied to the deposition region heat sink in sufficient quantities to lower the temperature of that region below the dewpoint of the iodides present in the chamber, as evidenced by the formation of a condensate upon the surface of the substrate. When this occurs, the coolant flow is carefully diminished to allow the temperature at the deposition region to increase slowly. As the dewpoint temperature is passed, the condensate on the substrate 32 will disappear. This temperature, which may vary somewhat due to differences in proportions of source materials present and to dopant concentrations, etc., may

be determined within sufficient tolerances by reading the temperature of the heat sink 18 at the time the condensate disappears.

The deposition region temperature is allowed to increase only slightly (about 5 to 10° C.) above the indicated dewpoint and then the coolant flow is adjusted to hold a constant temperature. This temperature is considerably below that at the source region, as shown in the 3rd and 4th columns of Table I. Under these conditions, a monocrystal of composition controlled in accordance with the source ingot proportions, as explained earlier, and doped with the impurity provided, will be observed to grow on the substrate. If the conditions have been properly established, good uniformity of growth will be observed. The quality of the crystal is visually determined by noting uniform glossy growth over the entire surface of the substrate. If some condition occurs which interferes with the growth process, as evidenced by condensation occurring or growth of spurious crystallites, then minor compensating adjustments may be made in the temperature of the source and deposition regions by coolant control. It may, at times, be necessary to temporarily invert the temperatures of the two regions to reverse the growth process and remove imperfect growths. This can be readily accomplished with the novel apparatus provided in accordance with this invention. After such removal, the initial growing conditions are re-established as previously described.

At the end of the growing process, which may be from about 5 hours to 20 hours for monocrystal of about 0.5 gm., the furnace power is discontinued and the system is allowed to cool down. At this time, the flow of coolant to heat sink 18 is diminished and the deposition region is allowed to approach chamber temperature. Coolant is supplied to the source region heat sink 20 at this time to cool it down considerably faster than the remainder of the system. This action insures termination of growth at the substrate and causes all remaining reaction products to be precipitated at the source region to prevent possible contamination of the grown crystal.

The particulars of a number of actual growth processes which produced high quality monocrystals are shown in Table I. The figures shown in this table are to be considered as exemplary only and are not intended to limit the invention except insofar as it is limited by the claims.

It will be seen from the examples in the table that any desired composition in the  $In(As_xP_{1-x})$  system may be produced in the form of high quality homogeneous monocrystals.

TABLE I

| Sample      | Composition                 | Source Area Temp. During Growth (° C.) | Substrate Area Temp. During Growth (° C.) | Dopant Concentration in Crystal (carriers/cc.) | Crystal Resistivity (ohm-cm.) | Hall Constant (cc./coulomb) |
|-------------|-----------------------------|----------------------------------------|-------------------------------------------|------------------------------------------------|-------------------------------|-----------------------------|
| MRM 18..... | InAs.....                   |                                        |                                           |                                                |                               |                             |
| MRM 19..... | $In(As_{.82}P_{.18})$ ..... | 820                                    | 760                                       | $Te-3.9 \times 10^{19}$                        | $9.73 \times 10^{-4}$         | 0.161                       |
| MRM 20..... | $In(As_{.85}P_{.15})$ ..... | 840                                    | 760                                       | $Te-2.3 \times 10^{19}$                        | $9.74 \times 10^{-4}$         | 0.273                       |
|             |                             |                                        |                                           | $Te-3.3 \times 10^{19}$                        | $22.6 \times 10^{-4}$         | 0.192                       |
| MRM 21..... | $In(As_{.51}P_{.49})$ ..... | 820                                    | 785                                       | $Te-1.4 \times 10^{19}$                        | $5.79 \times 10^{-4}$         | 0.441                       |
| MRM 23..... | $In(As_{.79}P_{.21})$ ..... | 825 to 885                             | 760                                       | $Te-2.6 \times 10^{19}$                        | $13.7 \times 10^{-4}$         | 0.230                       |
| MRM 24..... | $In(As_{.37}P_{.63})$ ..... | 835                                    | 700                                       | $Te-1.8 \times 10^{19}$                        | $1.66 \times 10^{-4}$         | 0.336                       |
| MRM 25..... | $In(As_{.84}P_{.16})$ ..... | 860                                    | 780                                       | $Te-2.2 \times 10^{19}$                        | $6.34 \times 10^{-4}$         | 0.281                       |
| MRM 26..... | $In(As_{.41}P_{.59})$ ..... | 820                                    | 720                                       | $Te-1.4 \times 10^{19}$                        | $2.28 \times 10^{-4}$         | 0.445                       |
| MRM 28..... | $In(As_{.18}P_{.82})$ ..... | 820                                    | 605                                       | $Te-6.8 \times 10^{18}$                        | $6.65 \times 10^{-4}$         | 0.918                       |

In all of the examples of Table I the growth process was carried out under the general condition described hereinbefore. The substrate-to-source distance was varied slightly in some cases but was always less than one inch. This spacing was not found to be particularly critical.

As indicated earlier herein, only general control of the doping concentration is available when the dopant is free in the chamber 10. If more precise control is desired, a crystal may be grown from a pair of source crystals, one of which has been previously doped to a known extent, and the other of which is undoped. By varying the proportions of the doped and undoped source crystal, any dopant concentration may be achieved.

Diodes are fabricated from the crystals produced in accordance with this invention, in a known manner. A typical procedure for fabricating a diode such as the one shown in FIG. 3, from a crystal doped with n-type impurity is described below.

The substrate containing the grown homogeneous single crystal layer is first oriented by use of an X-ray diffractometer, for example, to enable the crystal to be cut to provide a surface along the (100) crystallographic plane. The crystal is ground and polished along this plane to provide a surface free of defects and imperfections. The surface will become the face 40 of the finished diode. After polishing, the crystal is washed, dried, and prepared for diffusion of a junction therein.

For diffusion, the crystal is sealed in a quartz container containing a small quantity of zinc arsenide, for example 2 mg. for a container of 6 cc., and the container is evacuated to about  $10^{-7}$  torr. The container is thereafter heated in a furnace at about 650° C. for a period of about two hours. During this period, the zinc diffuses into the crystal from the various surfaces including the polished (100) plane surface, forming a p-type region in the n-type crystal. A junction, shown at 42 in FIG. 3, parallel with the (100) plane is formed between the p and n regions at a depth of about 1 mil from the polished surface.

After diffusion, the crystal is ground to provide a surface along the (100) plane on the side of the crystal opposite the previously polished surface. This will become the surface 44 of the finished diode. The grinding is carried to a depth sufficient to insure removal of any p-type material created on that side of the material and to reduce the thickness between the opposed surfaces to the order of about 5 mils.

Following the grinding operation the crystal, now in the form of a 5 mil thick wafer, is again washed and dried and provided with ohmic metallic contacts 46 and 48 on the (100) plane surfaces 40 and 44 by any known means, for example, electroless deposition.

It is desirable that the finished diode have end surfaces 50 and 52 perpendicular to the junction which are optically flat and parallel to each other. The purpose of these surfaces is to reflect a portion of the radiation produced in the junction region and to reinforce the emission in a known manner. While these surfaces may be produced by grinding and polishing, it is preferable to produce them by cleaving the crystal along the (110) crystallographic plane. The wafer is cleaved to provide two end surfaces along the (110) plane spaced about 17 mils apart.

The two side edges 54 and 56 of the finished diode are produced by sawing.

The completed diode shown on FIG. 3, is provided with suitable electrical conductors 58 and 60 which are attached to the ohmic contact surfaces 46 and 48, to provide means for injecting carriers therein.

Diodes fabricated as just described are operated as radiation emitting devices by injecting current thereto via the electrodes from a power source 62. Spontaneous emission of radiation from these diodes has been achieved with injection current densities as low as 525 amp per square centimeter at temperatures of 77° K. and at injection

tion current densities of 600 amp/cm.<sup>2</sup> at room temperature.

Stimulated emission, or true laser action, is achieved with current densities of as low as 6400 amps per square centimeter at temperatures of 77° K. for a typical sample. Both spontaneous and stimulated emission have been obtained in the absence of any magnetic field.

Table II gives data relating to actual operation of diodes fabricated from crystals grown in accordance with this invention. In Table II the leftmost column indicates the crystal sample from which the diode was fabricated. Table I gives the growth information concerning that sample.

TABLE II

| Sample | Diode<br>Temp.<br>(° K.) | Spontaneous Emission Data                   |                                      |                         |                                             | Stimulated Emission Data             |                         |       |  |
|--------|--------------------------|---------------------------------------------|--------------------------------------|-------------------------|---------------------------------------------|--------------------------------------|-------------------------|-------|--|
|        |                          | Current<br>Density<br>amp./cm. <sup>2</sup> | Line Max.<br>Wavelength<br>(microns) | Line Width<br>(microns) | Current<br>Density<br>amp./cm. <sup>2</sup> | Line Max.<br>Wavelength<br>(microns) | Line Width<br>(microns) |       |  |
| MRM 18 | 77                       | 1,050                                       | 3.25                                 | 0.24                    | -----                                       | -----                                | -----                   |       |  |
| MRM 19 | 77                       | 2,820                                       | 2.27                                 | 0.12                    | -----                                       | -----                                | -----                   |       |  |
| MRM 19 | 4                        | 3,300                                       | 2.23                                 | 0.08                    | -----                                       | -----                                | -----                   |       |  |
| MRM 20 | 4                        | 2,400                                       | 2.47                                 | 0.13                    | -----                                       | -----                                | -----                   |       |  |
| MRM 21 | 300                      | 600                                         | 1.71                                 | 0.18                    | -----                                       | -----                                | -----                   |       |  |
| MRM 21 | 77                       | 525                                         | 1.61                                 | 0.06                    | 15,400                                      | 1.60                                 | 0.0023                  | ----- |  |
| MRM 21 | 4                        | 4,000                                       | 1.59                                 | 0.02                    | 2,500                                       | 1.59                                 | 0.0051                  | ----- |  |
| MRM 21 | 2                        | -----                                       | -----                                | 620                     | 1.59                                        | 0.0004                               | -----                   | ----- |  |
| MRM 23 | 4                        | 1,200                                       | 2.19                                 | 0.09                    | -----                                       | -----                                | -----                   |       |  |
| MRM 25 | 4                        | 3,900                                       | 2.33                                 | 0.14                    | -----                                       | -----                                | -----                   |       |  |
| MRM 26 | 77                       | 1,500                                       | 1.44                                 | 0.05                    | 14,700                                      | 1.44                                 | 0.0064                  | ----- |  |
| MRM 26 | 4                        | -----                                       | -----                                | 35,600                  | 1.43                                        | 0.0052                               | -----                   | ----- |  |

For all samples shown in the table above, the spontaneous emission was produced by injection current in the form of pulses having a duration of 10 microseconds and a repetition rate of 500 pulses per second.

Stimulated emission for all tests of sample MRM26 and for the 77° K. test of MRM 21 was produced by injection current pulses having a duration of 50 nanoseconds and a repetition rate of 60 pulses per second. In the 4° K. and 2° K. tests of MRM21 pulses of 500 nanoseconds duration and a repetition rate of 100 p.p.s. were employed.

Examination of Table II shows the wide range of radiation wavelengths that are obtained with diodes provided in accordance with this invention. While data was not obtained for stimulated emission in all cases, the several examples of laser action which are given indicate the presence of a substantial range.

It will be noted that the line width obtained for the laser beam of the diode of MRM21 material when operated at 2° K. is extremely narrow. Since the wavelength of this material corresponds with one of the atmospheric windows in the infrared, it may be expected to be of significant importance.

It is also interesting to note that the MRM21 diode displayed spontaneous emission at a reasonable current density at room temperature. The ability to emit light at this temperature is unique and, of course, of considerable importance.

FIG. 4 of the drawings illustrates the emission characteristics of the MRM21 diode at 77° K. It will be observed that the spontaneous emission distribution curve 64 has the characteristic bell shape. The line width for spontaneous emission is about 600 Angstrom units. When the stimulated emission threshold is passed, the line narrows significantly (to about 23 Angstrom) as shown by curve 66, and the peak intensity goes up considerably.

FIG. 5 of the drawings illustrates the peak wavelengths of the various crystals grown in accordance with this invention. As shown in the chart, a substantially complete spectra of wavelengths between the InAs and InP wavelengths is provided. Any selected radiation wavelength may be obtained simply by adjusting the As:P ratio in the crystal grown in accordance with this invention.

It is believed to be apparent from the foregoing that the present invention provides the capability of producing high quality homogeneous monocrystals of controlled composition from which radiation emitting diodes may be fabricated. The means and methods for providing such

crystals are unique in the provision of independent control of the conditions at the source and substrate regions of the growth chamber, so that precleaning of the substrate is possible, so that low temperature reaction products may be kept away from the substrate both during the heat-up and cooling phases of the growth process, and so that conditions may be adjusted during growth. Another unique feature resides in the ability to view the process throughout its duration to monitor the growth and determine the actions to be taken to maintain optimum growth conditions. Another unique feature of the growth process resides in the recognition that growth of

In(As<sub>x</sub>P<sub>1-x</sub>) compounds is best achieved when the substrate region temperature is only slightly above the dew-point of the species present in that region of the chamber.

While the process has been described as employing iodine as the transfer agent, and indium, arsenic and phosphorus as the growth elements it will be understood that other halogen elements may be employed for transport, and that other III and IV group elements may be grown.

While the invention has been particularly shown and described with reference to preferred embodiments thereof, it will be understood by those skilled in the art that the foregoing and other changes in form and details may be made therein without departing from the spirit and scope of the invention.

What is claimed is:

1. A method of vapor growing a homogeneous monocrystal of controlled composition in III and V valence groups comprising:

enclosing source materials containing elements to be grown into said monocrystals in an evacuated chamber with a growth receiving substrate and a predetermined quantity of a halogen transport medium; heating said chamber to a temperature at which a halogen disproportionation reaction takes place; then lowering the temperature of the substrate to the dewpoint of the halides present in the chamber whereby condensate is detectable on the surface of the substrate;

then slowly increasing the temperature of the substrate to less than 10° C. above the dewpoint temperature whereby condensate is caused to disappear; then maintaining the substrate at said temperature above the dewpoint temperature, at which a uniform glossy appearance is observed over the entire surface of the substrate until a crystal of desired size has been deposited on the substrate.

2. A method of vapor growing a homogeneous crystal in accordance with claim 1 in which said method further includes:

discontinuing heating of said chamber and allowing it to cool, terminating temperature control of said substrate whereby the temperature rises to the temperature of said chamber, and lowering the temperature of the source materials below the temperature of the substrate whereby crystal growth on said substrate is terminated and any remaining reaction products in said chamber are caused to become deposited on said source materials.

3. A method of growing a homogeneous monocrystal in accordance with claim 1 wherein a predetermined amount of a selected semiconductor impurity element is enclosed in said chamber to cause said grown crystal to include a predetermined impurity concentration.

4. A method of growing a homogeneous monocrystal in accordance with claim 1 in which said source materials are ingots and wherein the areas of the surfaces of the ingots facing the substrate are arranged to have the same proportion that the elements in those ingots are desired to have in the grown crystal.

5. A method of growing homogeneous monocrystals in accordance with claim 4 where the ingots contain the elements indium, arsenic and phosphorus.

6. A method of vapor growing a homogeneous monocrystal in accordance with claim 4 in which:

20 said temperature of said chamber is between 750° C. and 900° C.;

said source materials are ingots comprised of indium arsenide and indium phosphide; and

25 said substrate is a monocrystal of indium arsenide.

7. A method of vapor growing a homogeneous monocrystal of the composition  $In(As_xP_{1-x})$ , where  $x$  is a selected value greater than zero and less than one, said method comprising:

enclosing ingots containing indium, arsenic, and phosphorus in an evacuated chamber with a growth receiving substrate and a predetermined quantity of iodine;

heating said chamber to a temperature between about 25 750° C. and 900° C.;

first controlling the temperature of the region of the chamber containing the ingots so that it remains substantially below the temperature of the substrate containing region of the chamber to cause the sur-

5

10

20

25

30

35

faces of the substrate to be etched and to insure that spurious reaction products are not deposited upon the substrate;

then allowing the temperature of the ingot containing region of the chamber to approach the temperature to which the chamber is heated and controlling the temperature of the region of the chamber containing the substrate to reduce it sufficiently below the chamber temperature to produce a condensate upon the substrate; and then raising the temperature of the region of the chamber containing the substrate until the condensate disappears and maintaining the region containing the substrate at a temperature up to 10° C. above the temperature which the condensate disappears, until a crystal of desired size has been deposited upon the substrate.

#### References Cited

#### UNITED STATES PATENTS

|           |         |                 |         |
|-----------|---------|-----------------|---------|
| 3,148,094 | 9/1964  | Kendall         | 148—175 |
| 3,218,205 | 11/1965 | Ruehrwein       | 148—175 |
| 3,224,911 | 12/1965 | Williams et al. | 148—175 |
| 3,224,913 | 12/1965 | Ruehrwein       | 148—175 |

#### OTHER REFERENCES

Marinace IBM Technical Disclosure Bulletin, vol. 3, No. 8, January 1961, p. 33.

HYLAND BIZOT, Primary Examiner.

DAVID L. RECK, JEWELL H. PEDERSEN, Examiners.

N. F. MARKVA, P. R. MILLER, P. WEINSTEIN, Assistant Examiners.